

June 19, 1945.

H. J. THIELKER

2,378,598

METHOD OF COATING

Filed Sept. 16, 1942

FIG. 1



→ 10

FIG. 2



FIG. 3



INVENTOR  
H. J. THIELKER

BY  
E.R. Nowlan  
ATTORNEY

## UNITED STATES PATENT OFFICE

2,378,598

## METHOD OF COATING

Henry J. Thielker, New York, N. Y., assignor to  
 Western Electric Company, Incorporated, New  
 York, N. Y., a corporation of New York

Application September 16, 1942, Serial No. 458,505

3 Claims. (Cl. 117—103)

This invention relates to a method of coating, and more particularly to a method of coating non-metallic articles having a rough surface, to create or restore a smooth surface thereon.

In the operation and maintenance of telephone apparatus it is found that those receiver and handset casings, for example, which are molded shells of phenol-formaldehyde condensation resins, may under certain conditions in time come to have their smooth outer surfaces etched into dull roughness by the natural exudations of the hands of the users. The original polish of the surface of such an article derives from its having been molded against the highly polished surface of a hot metal mold. When once this highly polished skin is dulled by abrasion or corrosion, it is not practicably possible to restore it by any mechanical method of grinding and polishing. Any ordinary type of paint or enamel does not, in most cases at least, have sufficient adhesion to the artificial resins, of which not only some telephone receiver and handset housings are made but also other articles of innumerable variety, and subject also to abrasive or corrosive wear.

An object of the invention is to provide a method of coating articles and especially non-metallic articles of molded artificial resin with a coating to provide originally or to restore a smooth surface to such articles having a matt, roughened or even indented or pitted surface.

With the above and other objects in view, the invention may be embodied in particular steps of suitably cleaning the surface of an article to be treated, preparing a solution of a partially condensed artificial resin condensation product in a volatile solvent, coating the cleaned article with the coating material so prepared, and heating the coated article to both drive off the solvent and complete the condensation of the resin on the surface.

Other objects and features will appear from the following detailed description of one embodiment of the invention taken in connection with the accompanying drawing, in which the same reference numerals are applied to identical parts in the several figures and in which

Fig. 1 is a diagrammatic view in perspective of the essentials of a tumbling barrel employable in carrying out the method of the invention;

Fig. 2 is a partial sectional view of a modified form thereof taken on the line 2—2 of Fig. 1; and

Fig. 3 is a perspective view of one of the tumbling pegs employed in the barrel.

The invention will be herein disclosed as em-

ployed for the restoring of a polished outer surface to the phenol-formaldehyde resin molded casings or housings of telephone receivers which have become matt or even pitted by abrasion, corrosion or both, in use. It will be remembered, however, that there is only one specific illustrative case of use of the invention among an innumerable number of analogous cases, as will be hereinafter indicated.

10 In carrying out the invention, as herein illustratively disclosed, there is employed a particular composition of matter. The particular telephone parts in question are moldings of a mixture comprising primarily a phenol-formaldehyde condensation resin, e. g. "Bakelite," "Catalin" or the like commercially named material, in fully and irreversibly condensed solid form. To coat these abraded or corroded articles, there is employed a commercially available partially condensed phenol-formaldehyde material. This is a clear, substantially colorless, sirupy liquid primarily intended for molding by casting in hot molds without pressure, and which will stay in storage at ordinary temperatures 20 (say not over 80° F.) substantially unchanged for a considerable length of time (say six months) but which when heated to about 130°—180° F., will become completely condensed into a solid, irreversible resin. In practise, the time required 30 for this final condensation is shortened if a suitable proportion of an accelerator such as hydrochloric acid is added thereto.

One such product is commercially known as "Catabond 200 CZ" and is manufactured for sale 35 by the Catalin Corporation of New York City. For applicant's present purpose a mixture is made up substantially as follows:

## Coating mixture I

40 Catabond 200 CZ \_\_\_\_\_ grams 170  
 Alcohol (ethyl, 95%) \_\_\_\_\_ cubic centimeters 96  
 Hydrochloric acid (35%) \_\_\_\_\_ do 9

This mixture is rendered sufficiently thin and 45 flowable at ordinary temperatures by the alcohol added to be applied by the method herein-after described. A coating of the mixture having been applied, the coated article is heated as hereinafter described for from thirty to ninety 50 minutes at a temperature preferably about 140° F. at first and rising to about 170° F. toward the end of the heating period, when the alcohol and water will have been wholly driven off together with the hydrogen chloride gas or the ammonium 55 chloride formed, and the coating will have set

into a remarkably strongly adherent, solid film with a highly polished and hard and resistant surface.

In handling a considerable number of articles to be coated, especially of irregular form such as molded telephone parts, applicant prefers the following process employing a tumbling barrel whose essentials are represented in the accompanying drawing, only those elements being shown which are essential for an understanding of the particular procedure involved. In this preferred procedure, the articles are

(1) Washed thoroughly, e. g. in soap and water, and rinsed.

(2) Degreased, e. g. with carbon tetrachloride liquid or vapor,

(3) Charged into a tumbling barrel with a suitable amount of the above described mixture of Catabond 200 CZ, alcohol and hydrochloric acid and with a suitable volume of waxed tumbling pegs, and the charging apertures of the barrel closed with impervious doors,

(4) Tumbled at room temperature for ten to fifteen minutes,

(5) Tumbled at about 140° F. for about thirty minutes, and

(6) Tumbled for about sixty minutes with the heat supply cut off and with multiperforate doors substituted for the impervious doors.

Articles of almost any artificial resin, of vulcanized hard rubber, of hard fiber, of wood, or of other generally analogous, not principally metallic material, after being subjected to the above procedure, are found to have a complete, remarkably strongly adherent and highly polished coating.

During the fifth step above, of tumbling at 140° F. with the barrel loading apertures closed with impervious doors, the further condensation of the partially condensed resin in the raw coating begins, but proceeds slowly enough so that the volatile solvent may be driven off without producing permanent pits or bubbles in the gradually hardening material, whose liquidity and surface tension remain sufficient to keep the surface of the coating smooth until the major portion, perhaps substantially all of the solvent has been driven out. With the impervious doors, the solvent vapors remain in the barrel and increase in density, so that the rapidity with which the solvent leaves the coating and hence the tendency to produce bubbles diminish as the material of the coating thickens and becomes more liable to bubble damage. By the end of the thirty minutes of this step there is not enough solvent left in the partially hardened coating to do any damage by its evaporation. The temperature is raised then for the sixth step to hasten the final setting of the coating, and the impervious doors are replaced by the easily pervious screen doors to allow the solvent vapors to escape and thus lower the vapor pressure of the solvent in the barrel to let the last traces of solvent be driven out of the coating freely.

As indicated in the drawing, the tumbling barrel, generally indicated at 10, may be a hollow, horizontal, polygonal prism of wood or other suitable material, journaled as indicated at 11 to be rotatably driven by means (not shown) about its horizontal axis. One side, 12, or two opposite sides 12 and 13 have suitable loading apertures 14, 14, which may be closed by removable solid doors 15 or by doors 115 (Fig. 2) having large apertures therein covered with

woven wire screens 16. The pegs 17, of which one of suitable form is shown on an enlarged scale in Fig. 3, are preferably of hard wood, e. g. maple, having the form shown in Fig. 3, although the particular form and material are not critical, so long as the pegs are somewhat porous and can be impregnated with waxy material, e. g. paraffin, to prevent the coating material from adhering to them in any substantial amount. For providing heat, the barrel may also be furnished with one or more longitudinally disposed elements 18 which may be heated by any suitable means (not shown), e. g. electrically or by circulation of hot liquid or vapor through them.

If a less highly polished but smooth surface be desired, a commercial product consisting essentially of the same sirupy, partially condensed phenol-formaldehyde compound, but containing about thirty per cent (30%) by weight of a mineral filler in highly divided form, may be employed to make a suitable coating mixture. A satisfactorily partially condensed resin plus mineral filler is the product manufactured by the Catalin Corporation for sale under the commercial name of "Catabond 3C," which is the same material above described and designated "Catabond 200 CZ" with about thirty percent (30%) of mineral filler added. A suitable coating mixture may be as follows:

#### Coating mixture II

|                                   |                   |     |
|-----------------------------------|-------------------|-----|
| Catabond 3C-----                  | grams             | 170 |
| Alcohol (as above)-----           | cubic centimeters | 19  |
| Hydrochloric acid (as above)----- | do                | 9   |

This mixture applied in a tumbling barrel as above described, produces a hard, smooth, remarkably strongly adherent coating, similar to that produced by the first mixture described, but distinctly less shiny although by no means dullly matt.

By adding two grams of aluminum stearate to the last mixture above, the coatings obtained will be definitely "flat" or matt. The mixture will then be

#### Coating mixture III

|                                   |                   |     |
|-----------------------------------|-------------------|-----|
| Catabond 3C-----                  | grams             | 170 |
| Alcohol (as above)-----           | cubic centimeters | 19  |
| Hydrochloric acid (as above)----- | do                | 9   |
| Aluminum stearate-----            | grams             | 2   |

Any of the coating compositions above described may, of course, have suitable pigments added to them to give the final coating a desired color.

With none of the above coating compositions and methods is any kind of preliminary filler coating, primer coating or other preliminary coating required; and in most instances such a preliminary coating is not even tolerable, if the final coating is to have the remarkably firm adhesion to an under body of artificial resin, hard rubber, hard fiber, wood or the like materials, which is characteristic of the coatings of the invention. The mixtures and procedures described do not, however, produce satisfactorily adherent coatings on metallic surfaces unless these are pre-coated in such a way as to be no longer characteristically metallic. The invention has been described and illustrated particularly in connection with articles of phenol-formaldehyde resin. It has not been tried out on all the vast variety of new thermosetting molding plastics which have been and are right along appearing in use. It will not, in general, be

applicable in the case of articles made of the thermoplastic resins such as the polymerization products of vinylidene, butylene and the like. However, it is believed to be applicable to articles made of any of the thermosetting compositions based on condensation products of phenol, cresol, and the like with formaldehyde, acetaldehyde, urea, furfural, glyptal and the like. Other volatile solvents besides ethyl alcohol, e. g. acetone, may be used in appropriate cases and other accelerators than hydrochloric acid, e. g. phosphoric acid or a suitable acid salt, although hydrochloric acid is preferable.

What is claimed is:

1. The method of coating the entire suitably clean outer non-metallic surface of articles which comprises steps of charging into a tumbling barrel provided with means to render a wall portion thereof pervious or impervious at will, the articles to be coated and a supply of waxed tumbling pegs together with a proportion of a raw coating composition containing a partially condensed condensation resin in liquid form and a volatile solvent therefor and an accelerator, tumbling the contents of the barrel therein at room temperature to coat the outer surface of the articles completely with the composition, continuing the tumbling of the contents of the barrel therein while heating the interior thereof to a temperature at which the volatile solvent is removed in major part before the condensation of the partially condensed resin has progressed materially, the walls of the barrel being wholly impervious during this step to prevent escape of the vapors of the evaporated solvent from the neighborhood of the coated surfaces of the articles to thereby aid in slackening the rate of escape of the solvent from the coated surfaces of the articles, rendering a wall portion of the barrel pervious, and continuing the tumbling of the contents of the barrel therein while heating the interior thereof to a higher temperature to complete the condensation of the resin and to remove substantially all of the solvent, the barrel being provided with a pervious wall portion during this step to release the entrapped vapors of the evaporated solvent from the neighborhood of the coated surfaces of the article to thereby promote the escape of the last traces of solvent from the heated coatings.

2. The method of coating the entire suitably clean outer non-metallic surface of articles which comprises steps of charging into a tumbling barrel provided with means to render a wall portion thereof pervious or impervious at will, the articles to be coated and a supply of waxed tumbling pegs together with a proportion of a raw coating composition containing a partially condensed phenol-formaldehyde resin in liquid form and alcohol and hydrochloric acid, tumbling the contents of the barrel therein at room temperature to coat the outer surface of the articles completely with the composition, continuing the tumbling of the contents of the barrel therein while heating the interior thereof to a temperature of about 140° F. at which the alcohol is removed in major part before the condensation of the partially condensed resin has progressed materially, the walls of the barrel being wholly impervious during this step to prevent escape of the vapors of the evaporated alcohol from the neighborhood of the coated surfaces of the articles to thereby aid in slackening the rate of escape of the alcohol from the coated surfaces of the articles, rendering a wall portion of the barrel pervious, and continuing the tumbling of the contents of the barrel therein while heating the interior thereof to a higher temperature of about 170° F. to complete the condensation of the resin and to remove substantially all of the alcohol, the barrel being provided with a pervious wall portion during this step to release the entrapped vapors of the evaporated alcohol from the neighborhood of the coated surfaces of the articles to thereby promote the escape of the last traces of alcohol from the heated coatings.

5 the composition, continuing the tumbling of the contents of the barrel therein while heating the interior thereof to a temperature at which the alcohol is removed in major part before the condensation of the partially condensed resin has progressed materially, the walls of the barrel being wholly impervious during this step to prevent escape of the vapors of the evaporated alcohol from the neighborhood of the coated surfaces of the articles to thereby aid in slackening the rate of escape of the alcohol from the coated surfaces of the articles, rendering a wall portion of the barrel pervious, and continuing the tumbling of the contents of the barrel therein while heating the interior thereof to a higher temperature to complete the condensation of the resin and to remove substantially all of the alcohol, the barrel being provided with a pervious wall portion during this step to release the entrapped vapors of the evaporated alcohol from the neighborhood of the coated surfaces of the articles to thereby promote the escape of the last traces of alcohol from the heated coatings.

10 3. The method of coating the entire suitably clean outer non-metallic surface of articles which comprises steps of charging into a tumbling barrel provided with means to render a wall portion thereof pervious or impervious at will, the articles to be coated and a supply of waxed tumbling pegs together with a proportion of a raw coating composition containing a partially condensed phenol-formaldehyde resin in liquid form and alcohol and hydrochloric acid, tumbling the contents of the barrel therein at room temperature to coat the outer surface of the articles completely with the composition, continuing the tumbling of the contents of the barrel therein while heating the interior thereof to a temperature of about 140° F. at which the alcohol is removed in major part before the condensation of the partially condensed resin has progressed materially, the walls of the barrel being wholly impervious during this step to prevent escape of the vapors of the evaporated alcohol from the neighborhood of the coated surfaces of the articles to thereby aid in slackening the rate of escape of the alcohol from the coated surfaces of the articles, rendering a wall portion of the barrel pervious, and continuing the tumbling of the contents of the barrel therein while heating the interior thereof to a higher temperature of about 170° F. to complete the condensation of the resin and to remove substantially all of the alcohol, the barrel being provided with a pervious wall portion during this step to release the entrapped vapors of the evaporated alcohol from the neighborhood of the coated surfaces of the articles to thereby promote the escape of the last traces of alcohol from the heated coatings.

HENRY J. THIELKER.